



US006436830B1

(12) **United States Patent**  
Merchant et al.

(10) **Patent No.:** US 6,436,830 B1  
(45) **Date of Patent:** Aug. 20, 2002

(54) **CMP SYSTEM FOR POLISHING SEMICONDUCTOR WAFERS AND RELATED METHOD**

(75) Inventors: **Sailesh Mansinh Merchant; Sudhanshu Misra; Pradip Kumar Roy**, all of Orlando, FL (US)

(73) Assignee: **Agere Systems Guardian Corp.**, Orlando, FL (US)

(\*) Notice: Subject to any disclaimer, the term of this patent is extended or adjusted under 35 U.S.C. 154(b) by 0 days.

(21) Appl. No.: **09/413,741**

(22) Filed: **Oct. 6, 1999**

(51) **Int. Cl.<sup>7</sup>** ..... H01L 21/302

(52) **U.S. Cl.** ..... 438/692; 438/693; 216/88; 216/89

(58) **Field of Search** ..... 438/691-693, 438/700; 51/307, 308; 216/88, 89; 134/1-3

(56) **References Cited**

U.S. PATENT DOCUMENTS

5,366,542 A \* 11/1994 Yamada et al. ..... 106/3  
5,516,346 A \* 5/1996 Cadien et al. ..... 51/308  
5,662,769 A \* 9/1997 Schonauer et al. ..... 438/633

|             |        |                             |           |
|-------------|--------|-----------------------------|-----------|
| 5,728,308 A | 3/1998 | Muroyama .....              | 216/88    |
| 5,733,819 A | 3/1998 | Kodama et al. .....         | 438/692   |
| 5,916,819 A | *      | 6/1999 Skrovan et al. ..... | 438/692   |
| 5,916,855 A | 6/1999 | Avanzino et al. .....       | 51/307    |
| 6,027,669 A | 2/2000 | Miura et al. .....          | 252/518.1 |
| 6,099,394 A | *      | 8/2000 James et al. .....   | 451/72    |
| 6,117,783 A | 9/2000 | Small et al. .....          | 438/693   |
| 6,136,714 A | *      | 10/2000 Schutz .....        | 438/692   |
| 6,140,130 A | *      | 10/2000 Salmen et al. ..... | 436/55    |

\* cited by examiner

*Primary Examiner*—Benjamin L. Utech

*Assistant Examiner*—Duy-Vu Deo

(57) **ABSTRACT**

A chemical mechanical polishing (CMP) system includes a polishing device including a polishing article. The polishing device holds the semiconductor wafer and provides relative movement between the semiconductor wafer and the polishing article with a slurry therebetween. The CMP system also includes a slurry processor for processing used slurry from the polishing device and for delivering processed slurry to the polishing device. The slurry processor including a metal separator for separating metal particles, polished from the semiconductor wafer, from the used slurry. The slurry can be continuously recirculated during a CMP process without damaging and/or contaminating the layers of the semiconductor wafer.

**24 Claims, 4 Drawing Sheets**



FIG. 1



FIG. 2



FIG. 3





**CM P SYSTEM FOR POLISHING  
SEMICONDUCTOR WAFERS AND RELATED  
METHOD**

**FIELD OF THE INVENTION**

The present invention relates to semiconductor processing, and, more particularly, to planarizing or polishing semiconductor wafer surfaces during the manufacture of integrated circuits.

**BACKGROUND OF THE INVENTION**

Semiconductor devices, also called integrated circuits, are mass produced by fabricating of identical circuit patterns on a single semiconductor wafer. During the process, the wafer is cut into identical dies or chips. Although commonly referred to as semiconductor devices, the devices are fabricated from various materials, including conductors (e.g. copper, aluminum and tungsten), non-conductors (e.g. silicon dioxide) and semiconductors (e.g. silicon). Silicon is the most commonly used semiconductor, and is used in either its single crystal or polycrystalline form. Polycrystalline silicon is often referred to as polysilicon or "poly". The conductivity of the silicon is adjusted by adding impurities in a process commonly referred to as doping.

Within an integrated circuit, thousands of devices (e.g., transistors, diodes) are formed. Typically, contacts are formed where a device interfaces to an area of doped silicon. Specifically, plugs are typically formed to connect metal layers with device active regions. Vias are typically formed to connect metal layers with other metal layers. Also interconnects are typically formed to serve as wiring lines to interconnect the many devices on the integrated circuit and the many regions within an individual device. These contacts and interconnects are formed using conductive materials.

The integrated circuit devices with their various conductive layers, semiconductive layers, insulating layers, contacts and interconnects are formed by fabrication processes, including doping processes, deposition processes, photolithographic processes, etching processes and other processes. At certain steps, it is often desirable to achieve a pre-determined level of surface planarity uniformity, and/or roughness. It is also desirable to minimize surface defects such as pits and scratches. Such surface irregularities may affect the performance of the final semiconductor device and/or create problems during subsequent processing steps.

One common technique to planarize a wafer is known as chemical mechanical polishing (CMP). CMP is very widely used technique which delivers a slurry of material to the wafer surface and while a polishing pad or belt is passed over the wafer surface. The slurry typically includes a plurality of abrasive particles dispersed in a liquid. For example, U.S. Pat. No. 5,728,308 entitled "Method of polishing a semiconductor substrate during production of a semiconductor device" discloses a conventional slurry used for chemical mechanical polishing including particulates comprised of metal oxides such as silica ( $SiO_2$ ), alumina ( $Al_2O_3$ ), titanium oxide ( $TiO_2$ ), and cerium oxide ( $CeO_2$ ) of a particle size of about 10 nm in an aqueous solution of potassium hydroxide (KOH).

A problem with current CMP slurries is that polished metal in the slurry can cause scratches on the wafer surface or contaminate layers on the wafer. Therefore, the slurry is not re-usable and increases waste.

**SUMMARY OF THE INVENTION**

In view of the foregoing background, it is therefore an object of the present invention to remove metal particles

from a slurry during CMP to avoid damaging and/or contaminating the semiconductor wafer.

It is another object of the present invention to provide a system which can process and re-use a slurry during CMP.

5 These and other objects, features and advantages in accordance with the present invention are provided by a chemical mechanical polishing (CMP) system including a polishing device having a polishing article for relative movement with the semiconductor wafer and with a slurry therebetween. The system further includes a slurry processor for processing used slurry from the polishing device and for delivering processed slurry to the polishing device. The slurry processor comprising a metal separator for separating metal particles, polished from the semiconductor wafer, from the used slurry. The slurry can be continuously recirculated during a CMP process without damaging and/or contaminating the layers of the semiconductor wafer.

10 The slurry preferably comprises a first emulsion including a continuous aqueous phase and a second emulsion. The second emulsion capturing metal particles polished from the semiconductor wafer. The slurry processor preferably comprises a first de-emulsifier for de-emulsifying the first emulsion into the continuous aqueous phase and the second emulsion. Furthermore, the second emulsion preferably 15 comprises an organic phase and a dispersed aqueous phase. The dispersed aqueous phase capturing the metal particles polished from the semiconductor wafer. The slurry processor preferably includes a second de-emulsifier for de-emulsifying the second emulsion into the organic phase and the dispersed aqueous phase, and for providing the dispersed aqueous phase with captured metal particles to the metal separator.

20 Also, the slurry processor may include an emulsifier for emulsifying the dispersed aqueous phase in the organic phase to form the second emulsion, and for emulsifying the second emulsion in the continuous aqueous phase to form the first emulsion. The metal separator provides the dispersed aqueous phase without captured metal particles to the emulsifier, and the emulsifier delivers processed slurry to the 25 polishing device.

25 The objects, features and advantages in accordance with the present invention are also provided by a method of chemical mechanical polishing including delivering a slurry to an interface between a semiconductor wafer and a polishing article while providing relative movement therebetween. The slurry preferably comprises a first emulsion including a continuous aqueous phase and a second emulsion. The second emulsion captures metal particles polished from the semiconductor wafer.

30 The method preferably further includes collecting used slurry from the interface between the semiconductor wafer and the polishing article, processing the used slurry, and delivering the processed slurry to the interface between the semiconductor wafer and the polishing article. The second emulsion may include an organic phase and a dispersed aqueous phase, the dispersed aqueous phase capturing the metal particles polished from the semiconductor wafer. Also, the step of processing the used slurry preferably includes de-emulsifying the first emulsion into the continuous aqueous phase and the second emulsion, de-emulsifying the second emulsion into the organic phase and the dispersed aqueous phase, and removing captured metal particles from the dispersed aqueous phase. The step of processing the used slurry may also include emulsifying the dispersed aqueous phase in the organic phase to form the second emulsion, and emulsifying the second emulsion in the continuous aqueous phase to form the first emulsion.

The continuous aqueous phase may include abrasive particles and the dispersed aqueous phase may comprise a dispersed aqueous acidic phase. The organic phase may comprise an alcohol or iso-alcohol and may include at least one complexing agent for reacting with metal particles polished from the semiconductor wafer to form organometallic complexes. The complexing agent may comprise at least one of ethylene diamine tetra-acetate (edta), di-ethylene triamine penta-acidic acid (dtpa), 8-hydroxy quinoline, bi-pyridine, and ortho-phenanthroline. The organic phase transports the organometallic complexes to an interface between the organic phase and the dispersed aqueous phase by diffusion. The organometallic complexes decompose at the interface to release the complexing agent into the organic phase and release the metal particles into the dispersed aqueous phase.

#### BRIEF DESCRIPTION OF THE DRAWINGS

FIG. 1 is a schematic view of a CMP slurry at the interface of a semiconductor wafer and a polishing article in accordance with the present invention.

FIG. 2 is an enlarged schematic view of the CMP slurry to schematically illustrate movement of metal across the first and second emulsions in accordance with the present invention.

FIG. 3 is a flowchart illustrating the basic steps of chemically mechanically polishing using a slurry in accordance with the present invention.

FIG. 4 is a schematic diagram of a CMP system for processing used slurry in accordance with the present invention.

#### DETAILED DESCRIPTION OF THE PREFERRED EMBODIMENTS

The present invention will now be described more fully hereinafter with reference to the accompanying drawings, in which preferred embodiments of the invention are shown. This invention may, however, be embodied in many different forms and should not be construed as limited to the embodiments set forth herein. Rather, these embodiments are provided so that this disclosure will be thorough and complete, and will fully convey the scope of the invention to those skilled in the art. Like numbers refer to like elements throughout. The dimensions of layers and regions may be exaggerated in the figures for greater clarity.

Referring initially to FIG. 1, a CMP slurry 10 in accordance with the present invention will now be described. The CMP slurry 10 includes a first emulsion 11 having a continuous aqueous phase (AQ<sub>E</sub>) 12 and a second emulsion 13. An emulsion is a system including a liquid dispersed with or without an emulsifier in an immiscible liquid usually in droplets of larger than colloidal size. The first emulsion 11 includes abrasive particles 18 such as silica, alumina or ceria as would be appreciated by those skilled in the art. The second emulsion 13 preferably comprises an organic phase (ORG) 14 and a dispersed aqueous phase (AQ<sub>I</sub>) 16 for capturing metal particles polished from the semiconductor wafer 20.

The semiconductor wafer 20 includes a metal layer 22 which may include copper, tantalum, titanium, tantalum nitride or any other metal commonly used in the production of integrated circuits. Metal particles are polished off the metal layer 22 during a CMP process using the slurry 10 at an interface between the semiconductor wafer 20 and a polishing article 24, such as a pad or belt. Such metal

particles can damage and/or contaminate the semiconductor wafer as discussed above. The slurry 10 captures the metal particles in the second emulsion 13, which permits the removal of the metal particles and allows the slurry 10 to be continuously recirculated during the CMP process without damaging and/or contaminating the layers of the semiconductor wafer 20.

Referring additionally to FIG. 2, movement of the metal across the first and second emulsions 12, 14 will now be described in accordance with the present invention. The dispersed aqueous phase 16 is preferably a dispersed aqueous acidic phase. The organic phase 14 may comprise alcohol or iso-alcohol and preferably includes at least one complexing agent such as, for example, ethylene diamine tetra-acetate (edta), di-ethylene triamine penta-acidic acid (dtpa), 8-hydroxy quinoline, bi-pyridine, or ortho-phenanthroline, including ligand R, for reacting with metal particles polished from the metal layer 22 of semiconductor wafer 20 to form organometallic complexes. For example, di-ethylene triamine penta-acidic acid is particularly suitable for copper, tungsten or tantalum, 8-hydroxy quinoline is particularly suitable for aluminum, and bi-pyridine is particularly suitable for copper. As illustrated, the metal particles polished from the metal layer 22 may form, for example, copper ions Cu<sup>2+</sup> in the slurry 10. The copper ions Cu<sup>2+</sup> will readily form organometallic complexes Cu<sup>X</sup>R by chemical reaction with the complexing agent at the interface 26 between the continuous aqueous phase 12 and the organic phase 14.

The organic phase 14 then transports the organometallic complexes Cu<sup>X</sup>R to an interface 28 between the organic phase 14 and the dispersed aqueous phase 16 by diffusion. At this interface 28, the organometallic complexes Cu<sup>X</sup>R then decompose by chemical reaction to release the ligand R back into the organic phase 14 and release the copper ions Cu<sup>2+</sup> into the dispersed aqueous phase 16. The released ligand R of the complexing agent is then available for complexing reaction with the metal species, e.g. copper ions Cu<sup>2+</sup>, at the interface 28 between the organic phase 14 and the dispersed aqueous phase 16. This chemical reaction at the interface 28 between the organic phase 14 and the dispersed aqueous phase 16 results in a continuous chemical potential gradient across the organic phase that enhances the transport of the organometallic complexes Cu<sup>X</sup>R.

As mentioned above, the dispersed aqueous phase 16 may be an aqueous acidic dispersed phase, and the pH differences between the continuous aqueous phase 12 and the dispersed aqueous phase 16 can effect the chemical potential gradient for metal transport across the organic phase 14. By having a continuous driving force across the organic phase 14, the interface 26 will not be flooded with an influx of metal ions. The metal transport across the organic phase 14 will be diffusion limited, but will not be limited by the chemical complex formation and decomposition reactions at the interfaces 26, 28.

Referring now to FIGS. 3 and 4, a system 29 and a method for CMP, in accordance with the present invention, will now be described. Specifically, while referring to FIG. 3, the system 29 includes a slurry processor 30 and a polishing device 31. The polishing device 31 includes the polishing article 24, such as a pad or belt. The polishing device 31 provides relative movement between the semiconductor wafer 20 and the polishing article 24 with a slurry 10 therebetween. The wafer 20, the polishing article 24 or both may be rotated during CMP. The slurry processor 30 includes a first de-emulsifier 32 which receives the used slurry, a second de-emulsifier 33 downstream from the first

de-emulsifier, a metal separator **34** downstream from the second de-emulsifier, and an emulsifier **36** connected to both de-emulsifiers and the metal separator.

Referring to FIGS. 3 and 4, the method for CMP begins at Block **40** and a slurry **10** is delivered to the interface between the semiconductor wafer **20** and the polishing article **24** in the polishing device **31**. Here, the slurry **10** is preferably a multiple emulsion ((AQ<sub>f</sub>/ORG) /AQ<sub>E</sub>) as described above with reference to FIGS. 1 and 2. A second emulsion (AQ<sub>f</sub>/ORG) **13** is emulsified in a continuous aqueous phase (AQ<sub>E</sub>) **12** to define a first emulsion **11**. A dispersed aqueous phase (AQ<sub>f</sub>) **16** is emulsified in an organic phase ORG **14** to define the second emulsion **13**. Again, as described in detail above, the dispersed aqueous phase (AQ<sub>f</sub>) **16** captures metal particles, e.g. metal ions, polished from the semiconductor wafer **20**. Of course additives, abrasives, corrosion inhibitors etc., may be added to the continuous aqueous phase **12** of the slurry **10** as would be appreciated by the skilled artisan.

At Block **44**, the used slurry **10** containing the metal particles is collected and delivered to the first de-emulsifier **32** where it is de-emulsified (Block **46**) into the continuous aqueous phase **12** and the second emulsion **13**. The second emulsion **13** including the metal particles is delivered to the second de-emulsifier **33** where it is de-emulsified (Block **48**) into the organic phase **14** and the dispersed aqueous phase **16**. The dispersed aqueous phase **16** containing the metal particles is delivered to the metal separator **34** where the metal particles are removed (Block **50**) from the dispersed aqueous phase **16** and subsequently disposed at Block **52**.

The emulsifier **36** receives the organic phase from the second de-emulsifier **33** and receives the dispersed aqueous phase **16**, without the metal particles, from the metal separator **34**. The dispersed aqueous phase **16** is emulsified in the organic phase to re-form the second emulsion **13** in a first stage of emulsification (Block **54**). The emulsifier **36** also receives the continuous aqueous phase **12** from the first de-emulsifier **32**. The second emulsion **13** is then emulsified (Block **56**) in the continuous aqueous phase **12** to re-form the first emulsion **11** and complete the slurry **10**. The slurry **10**, as a multiple emulsion ((AQ<sub>f</sub>/ORG) /AQ<sub>E</sub>), is then recirculated into the loop and delivered to the polishing device **31**. Thus, as described, the slurry **10** can be continuously recirculated during a CMP process without damaging and/or contaminating the layers, e.g. metal layer **22**, of the semiconductor wafer **20**.

With respect to the emulsifier **36** and the first and second de-emulsifiers **32**, **33**, it is noted that emulsions may be prepared readily by shaking together the two liquids or by adding one phase drop by drop to the other phase with some form of agitation. Such agitation may include, for example, irradiation by high intensity ultrasonic waves. In a typical emulsifying device, the two liquids are forced through a narrow slit between a rapidly rotating rotor and a stator. The preparation of stable emulsions must be controlled carefully, because emulsions are sensitive to variations in the mode of agitation, the nature and amount of an emulsifying agent, and temperature changes. Emulsions may be de-emulsified in a number of ways including: addition of multivalent ions of a charge opposite to the emulsion droplet; chemical action; freezing; heating; aging; centrifuging; application of high-potential alternating electric fields; and treatment with low intensity ultrasonic waves.

Many modifications and other embodiments of the invention will come to the mind of one skilled in the art having the benefit of the teachings presented in the foregoing

descriptions and the associated drawings. Therefore, it is to be understood that the invention is not to be limited to the specific embodiments disclosed, and that modifications and embodiments are intended to be included within the scope of the appended claims.

That which is claimed is:

1. A method of chemical mechanical polishing (CMP) a semiconductor wafer including metal, the method comprising:

10 delivering a slurry to an interface between the semiconductor wafer and a polishing article while providing relative movement therebetween;

the slurry comprising a first emulsion including a continuous aqueous phase and a second emulsion, wherein the second emulsion captures metal particles polished from the semiconductor wafer.

2. A method according to claim 1, further comprising the steps of:

collecting used slurry from the interface between the semiconductor wafer and the polishing article;

processing the used slurry; and

delivering the processed slurry to the interface between the semiconductor wafer and the polishing article.

25 3. A method according to claim 2, wherein the step of processing the used slurry comprises at least one de-emulsifying step.

4. A method according to claim 2, wherein the step of processing the used slurry comprises removing captured metal particles from the slurry.

30 5. A method according to claim 2, wherein the step of processing the used slurry comprises:

de-emulsifying the first emulsion into the continuous aqueous phase and the second emulsion; and

removing captured metal particles from the second emulsion.

35 6. A method according to claim 2, wherein the second emulsion comprises an organic phase and a dispersed aqueous phase, the dispersed aqueous phase capturing the metal particles polished from the semiconductor wafer, and wherein the step of processing the used slurry comprises:

de-emulsifying the first emulsion into the continuous aqueous phase and the second emulsion;

de-emulsifying the second emulsion into the organic phase and the dispersed aqueous phase; and

removing captured metal particles from the dispersed aqueous phase.

40 7. A method according to claim 6, wherein the step of processing the used slurry further comprises:

emulsifying the dispersed aqueous phase in the organic phase to form the second emulsion; and

emulsifying the second emulsion in the continuous aqueous phase to form the first emulsion.

45 8. A method according to claim 1, wherein the continuous aqueous phase includes abrasive particles.

9. A method according to claim 6, wherein the dispersed aqueous phase comprises a dispersed aqueous acidic phase.

10. A method according to claim 6, wherein the organic phase comprises at least one of an alcohol and iso-alcohol.

11. A method according to claim 6, wherein the organic phase includes at least one complexing agent for reacting with metal particles polished from the semiconductor wafer to form organometallic complexes.

50 12. A method according to claim 11, wherein the at least one complexing agent comprises at least one of ethylene diamine tetra-acetate (edta), di-ethylene triamine penta-

acidic acid (dtpa), 8-hydroxy quinoline, bi-pyridine, and ortho-phenanthroline.

**13.** A method according to claim 11, wherein the organic phase transports the organometallic complexes to an interface between the organic phase and the dispersed aqueous phase by diffusion.

**14.** A method according to claim 13, wherein the organometallic complexes decompose at the interface to release the complexing agent into the organic phase and release the metal particles into the dispersed aqueous phase.

**15.** A method of chemical mechanical polishing (CMP) a semiconductor wafer including metal, the method comprising:

delivering a slurry to an interface between the semiconductor wafer and a polishing article while providing relative movement therebetween;

the slurry comprising a first emulsion including a continuous aqueous phase and a second emulsion, wherein the continuous aqueous phase includes abrasive particles, and wherein the second emulsion comprises an organic phase and a dispersed aqueous phase, the dispersed aqueous phase capturing metal particles polished from the semiconductor wafer.

**16.** A method according to claim 15, further comprising the steps of:

collecting used slurry from the interface between the semiconductor wafer and the polishing article;

processing the used slurry; and

delivering the processed slurry to the interface between the semiconductor wafer and the polishing article.

**17.** A method according to claim 16, wherein the step of processing the used slurry comprises at least one de-emulsifying step.

**18.** A method according to claim 16, wherein the step of processing the used slurry comprises removing captured metal particles from the slurry.

**19.** A method according to claim 16, wherein the step of processing the used slurry comprises:

de-emulsifying the first emulsion into the continuous aqueous phase and the second emulsion; and removing captured metal particles from the second emulsion.

**20.** A method according to claim 16, wherein the step of processing the used slurry comprises:

de-emulsifying the first emulsion into the continuous aqueous phase and the second emulsion;

de-emulsifying the second emulsion into the organic phase and the dispersed aqueous phase; and removing captured metal particles from the dispersed aqueous phase.

**21.** A method according to claim 20, wherein the step of processing the used slurry further comprises:

emulsifying the dispersed aqueous phase in the organic phase to form the second emulsion; and

emulsifying the second emulsion in the continuous aqueous phase to form the first emulsion.

**22.** A method according to claim 15, wherein the dispersed aqueous phase comprises a dispersed aqueous acidic phase.

**23.** A method according to claim 15, wherein the organic phase comprises at least one of an alcohol and and iso-alcohol.

**24.** A method according to claim 15, wherein the organic phase includes at least one complexing agent for reacting with metal particles polished from the semiconductor wafer to form organometallic complexes.

\* \* \* \* \*